

Dec. 25, 1923.

1,478,544

R. W. BIRD

SHINGLE STRIP

Filed Dec. 10, 1919



## UNITED STATES PATENT OFFICE.

REGINALD W. BIRD, OF FRAMINGHAM, MASSACHUSETTS, ASSIGNOR TO THE FLINT-KOTE COMPANY, OF BOSTON, MASSACHUSETTS, A CORPORATION OF MASSACHUSETTS.

## SHINGLE STRIP.

Application filed December 10, 1919. Serial No. 343,863.

To all whom it may concern:

Be it known that I, REGINALD W. BIRD, a citizen of the United States, residing at Framingham, in the county of Middlesex and State of Massachusetts, have invented new and useful Improvements in Shingle Strips, of which the following is a specification.

This invention has for its object to provide 10 a novel shingle strip, which, when laid with others in overlapping relation, produces the effect of spaced individual shingles.

In accordance with the present invention, 15 a sheet of felt, saturated or impregnated with an asphaltic or bituminous compound of relatively low melting point, is coated with a molten or plastic layer of higher-melting-point pitch or asphalt, and on the coating, while it is soft and plastic, is spread 20 a surface layer of crushed flaky slate or other mineral of the desired color, say red, green or brown. This layer is partially embedded by pressure in the asphaltic coating, so that the entire surface of the sheet is thus provided 25 with the mineral.

For the formation of the shingle strips to give them when laid the appearance of spaced individual shingles, the sheet is subjected to the pressure of a roll which is 30 provided with narrow ribs which act to embed the mineral material engaged thereby completely into the plastic coating so that the black coating appears and masks the mineral material. The sheet is then cut 35 along lines approximately perpendicular to the black lines or stripes so formed, such lines of severance being spaced apart a distance equal to the desired width of the strip. The operating roll may have circumferential 40 ribs, in which event the sheet is cut crosswise into strips, or else the ribs may extend longitudinally of its axis in which event the sheet is cut lengthwise, and is, at intervals, chopped off to give to the strips the desired 45 length.

On the accompanying drawings,—

Figure 1 represents conventionally and diagrammatically apparatus which may be employed in practicing my invention. 50 Figures 2 and 3 represent different forms of ribbed rolls for forming the stripes on the slate-surfaced sheet.

Figure 4 shows how the sheet is cut, when longitudinal pressure lines or stripes are 55 formed therein.

Figure 5 shows how the sheet is cut when transverse pressure lines are formed therein.

Figure 6 illustrates one of the strips.

Figure 7 represents in lengthwise section a portion of one of the shingle strips. 60

Figure 8 represents a portion of a roof covering comprising the strips laid in overlapping relation.

The sheet of felt 10 is drawn through a vat 11 containing the bituminous water-proofing compound, and, after passing between the cooling rolls 12, 12, is coated with asphalt or pitch at 13, in passing between the rolls 14, 14. The crushed flaky slate is supplied to the plastic coating by the hopper 15, 70 and, in passing between the rolls 16, 16, the slate is partially embedded therein, so that it entirely covers and conceals the bituminous coating. The operations, as thus far described, are those commonly followed in 75 making slate-surfaced roofing. After leaving the rolls 16, 16, with the coating still comparatively soft and plastic, the sheet is passed beneath a roll 17 which is provided with pressure ribs, equal in width to the 80

spaces which are ordinarily left between individual shingles when laid on the roof, to wit, about half an inch. The roll, which is preferably heated, may have circumferential ribs as at 18 in Figure 2 or longitudinal 85 ribs 19 as in Figure 3. These ribs are of such depth as to force the particles of slate engaged thereby into and completely embed them in the bituminous coating, so that they are covered and masked thereby, and, being 90 heated, soften the asphalt to assist in such embedment. The distance between the ribs is equal to the width of an ordinary shingle, e. g., five to six inches. If the black lines or stripes of depression are longitudinal of 95 the sheet, the sheet is cut transversely on the line *a*—*a*, Figure 4, so that each strip severed therefrom is equal in length to the width of the sheet, and in width is about 12 inches, or to the length of an individual 100 shingle. If the stripes of depression are transverse to the sheet as in Figure 5, the sheet is cut along the longitudinal lines *b*—*b* and is cut crosswise on the line *c*—*c*, thus producing shingle strips similar to those 105 produced from the sheet shown in Figure 4. The cutting machine is conventionally shown at 20 in Figure 1, and the sheet is shown as being festooned for cooling.

In the conventional illustration of the strip 110

in Figure 7, the saturated body of the strip is indicated at *e*, and the bituminous coating at *f*. The partially embedded slate is shown at *g*, while that which is wholly embedded 5 is indicated at *h*. Thus each strip, as shown in Figure 6, has the dark stripes or depressions *i* and the slate-surfaced bands *j*, which are approximately perpendicular to the top and bottom edges of the strip. When these 10 strips are placed in overlapping relation on a roof, as represented in Figure 8, the roof presents the appearance of one having individual spaced shingles thereon.

What I claim is:

13 1. A method of making shingle strips, adapted to be laid in overlapping relation in simulation of spaced individual shingles, consisting in partially embedding in the entire face of an asphalt-coated waterproofed 20 fibrous sheet a surface layer of colored crushed slate, then by pressure completely embedding portions of the slate in parallel spaced stripes into said asphaltic coating in contrast to the remainder of the slate-surfaced sheet, and then cutting said sheet 25 transversely of said stripes into strips each having a plurality of such stripes perpendicular to its greatest diameter.

2. A method of making shingle strips, adapted to be laid in overlapping relation in 20 simulation of spaced individual shingles, consisting in partially embedding in the entire face of an asphalt-coated waterproofed 25 fibrous sheet a surface layer of colored crushed slate, then by pressure completely embedding portions of the slate into the asphaltic coating in parallel stripes longitudinal of the sheet, and then severing said sheet transversely into strips of equal length, 30 with the stripes at an angle to the long edges 40 thereof.

3. A shingle strip, adapted to be laid with others in overlapping relation in simulation of spaced individual shingles, consisting of a waterproofed fibrous body having an 45 asphaltic coating, bands of colored crushed slate partially embedded in such coating to conceal the same, and intervening stripes in which the slate is completely embedded so as to be masked by the asphaltic coating, said 50 bands and contrasting intervening stripes being substantially perpendicular to the long top and bottom edges of the strip.

In testimony whereof I have affixed my signature.

REGINALD W. BIRD.